

April 8, 1930.

V. B. BROWNE

1,754,008

METHOD OF MAKING DUCTILE IRON CHROMIUM ALUMINUM ALLOYS

Filed Dec. 19, 1927



INVENTOR  
Vere B. Browne  
By Green and McCalister  
His Attorneys

## UNITED STATES PATENT OFFICE

VERE B. BROWNE, OF BRACKENRIDGE, PENNSYLVANIA

## METHOD OF MAKING DUCTILE IRON CHROMIUM ALUMINUM ALLOYS

Application filed December 19, 1927. Serial No. 241,208.

This invention relates to ferrous alloys and more particularly to alloys in which the principal elements aside from the iron are chromium and aluminum.

Many alloys containing iron, chromium and aluminum have from time to time been discussed in the technical literature and many such alloys are disclosed in patents. Many of these alloys show high electrical resistance and also high resistance to oxidation at elevated temperatures but as heretofore forged or otherwise worked, they have been practically valueless when ductility was necessary. These desirable inherent characteristics have caused much experimental work to be done by different researchers in an attempt to discover or provide a method of rendering the alloys ductile and readily workable.

The experimental work has covered a large number of alloys of this group and includes those having a chromium range of from 5% to 30% and an aluminum range of from 3% to 10%.

All alloys of this group having a chromium content ranging from 5% to 30% and an aluminum content ranging from 3% to 10%, when forged (which includes rolling) or otherwise worked under ordinary commercial methods develop an extremely large grain structure and this large grain structure cannot be transformed into a small grain structure by any known method of annealing. The large grain structure renders the finished product, that is, products made from these alloys so brittle, that their use in commercial work has been exceedingly limited and as a matter of fact where ductility has been necessary, it has been practically impossible to utilize them.

An object of this invention is to provide a method by means of which the brittle condition which has heretofore existed in alloys of this type can be avoided or overcome and whereby it is possible commercially to produce such alloys which are readily workable and from which may be produced articles such as wire, light gauge sheets, strips, etc., which are also relatively soft and ductile.

A further and more limited object of this

invention is to provide a method by means of which relatively soft, ductile resistor grids may be made from ferrous alloys containing from 5% to 30% of chromium and from 3% to 10% of aluminum, and in the drawings, I have shown in perspective view one of such grids.

I have discovered that these alloys develop an excessively large grain structure when heated to a temperature above 1500° F., and so far as I know, this large grain structure cannot be transformed into a small grain structure by any known method of annealing; I have found, however, that these alloys can be so worked as to render them relatively soft and ductile. This working in a broad way consists in forging at temperatures below 1500° F. and the best results can be obtained by carrying on the final reduction with the alloy in a relatively cold state and then by annealing the forged material below 1500° F.

I have carried on a large number of experiments with alloys having a chromium range of from 5% to 30% and an aluminum range of from 3% to 10%. I find that the alloy best suited (taking all things into consideration) for articles such as electrical resistance elements and articles that are to be subjected to elevated temperatures and must resist oxidation, is an alloy containing about 12% chromium and about 5% aluminum with the principal part of the remainder iron. The carbon should be kept low as possible and is preferably not over .12%.

These alloys are preferably manufactured in an electric arc furnace and the aluminum is preferably added just before teeming but if desired, may be added to the ladle.

In carrying out my method an ingot containing the desired percentages of iron, chromium and aluminum is heated to a temperature just high enough to permit it to be cogged or broken down into a bloom without rupturing its surface. The temperature which I have found satisfactory for this step is about 2000° F.

After the ingot is cogged or broken down, the bloom is reheated to approximately 1800°

F. and so rolled that the finishing passes take place at a temperature well below 1500° F.

Beginning at a stage in which the section is considerably larger than the finished section desired, all subsequent reductions are made at temperatures not exceeding 1500° F. Finishing is carried out below 1400° F. The final reduction is preferably made cold and I find that the best results are obtained when this is about 25%.

In a typical case involving my invention, I started with an ingot twelve inches square and weighing approximately twenty five hundred pounds. The analysis of this ingot was about 12% chromium, about 5% aluminum with the principal part of the remainder iron.

The ingot was heated to a temperature of about 2000° Fahrenheit and rolled to a billet about 5½ inches square. The billet was reheated to a temperature of about 1800° F. and rolled down to about 1¼ inches square. This square section was reheated to 1700° F. and rolled to a strip about 2½ inches wide by .072 inches thick and finished at a temperature of about 1400° F. The hot rolled strip .072 inches in thickness was then cold rolled to .040 inches in thickness and annealed at a temperature not exceeding 1450° F.

The material produced in this manner had a fine grain structure and was quite soft and ductile and readily workable.

It will be noted that each step of the forging or rolling operation was conducted at a lower temperature than the preceding step and that the final cold rolling represents a reduction of nearly 50%.

I prefer to carry on the final reduction with the material at room or atmospheric temperature, but fair results can be obtained if the temperature of the material does not exceed 1400° F.

What I claim is:

1. The method of making a ductile article from an iron chromium aluminum alloy having a chromium content of between about 10% and about 20%, an aluminum content between about 3% and about 10% with the remainder principally iron, which consists in casting an ingot of such alloy, in heating the ingot to a temperature of about 2000° F., in making material reductions by heating and rolling the same in successive steps in which the finishing temperatures decrease, in making the final reduction at about 1400° F. and then in annealing at a temperature of about 1400° F.

2. The method of making a ductile article from an iron chromium aluminum alloy having a chromium content of about 10-20%, an aluminum content of about 3-10% with the remainder principally iron, which consists in casting an ingot of such alloy, heating the ingot to about 2000° F., reducing the same materially by heating and rolling in successive steps at progressively

decreasing finishing temperatures, making a final material reduction at a temperature below 1400° F., and then annealing at about 1400° F.

3. The method of making a ductile article from an iron chromium aluminum alloy having a chromium content of about 10-20%, an aluminum content of about 3-10% with the remainder principally iron, which consists in casting an ingot of such alloy, heating the ingot to about 2000° F., reducing the same materially to a billet, reheating the billet to about 1800° F., reducing the so heated billet materially, reheating the reduced billet to about 1700° F., reducing the reheated reduced billet materially, finishing the same at about 1400° F., cold rolling to a materially reduced thickness, and annealing at not over about 1450° F.

In testimony whereof, I have hereunto subscribed my name this 15th day of December, 1927.

VERE B. BROWNE.

90

95

100

105

110

115

120

125

130